# EUROPEAN PATENT SPECIFICATION

(11) **EP 1 832 827 B1**
(45) Date of publication and mention of the grant of the patent: **20.08.2008**
(21) Application number: 07002322.1
(22) Date of filing: 02.02.2007
(51) Int. Cl.: F27D 9/00

(54) **Cooling apparatus for fired body, firing furnace, cooling method of ceramic fired body, and method for manufacturing honeycomb structured body**
Kühleinrichtung von keramischer Struktur, Ofen, Kühlverfahren und Verfahren zur Herstellung von Bienenwabenkörper aus Keramik
Dispositif de refroidissement, four de calcination, méthode de refroidissement et procédé de fabrication d'une structure céramique à nid d'abeille

(30) Priority: 08.03.2006 WO PCT/JP2006/304510
(43) Date of publication of application: 12.09.2007
(73) Proprietor: IBIDEN CO., LTD., Ogaki-shi Gifu 503-8604 (JP)
(72) Inventor: Kuribayashi, Koji Ibiden Co., Ltd., Ibi-gun Gifu 501-0695 (JP); Saijo, Takamitsu Ibiden Hungary KFT., 2326 Hungary (HU); Higuchi, Koji Ibiden Co., Ltd., Ibi-gun Gifu 501-0695 (JP)
(74) Representative: HOFFMANN EITLE

(56) References cited:
- EP-A- 1 696 194
- EP-A1- 0 576 934
- WO-A-20/06048003
- US-A- 4 364 760
- US-A- 4 927 577
- US-A- 5 183 609
- US-A- 6 089 860

## Description

### TECHNICAL FIELD

The present invention relates to a cooling apparatus for a fired body, a firing furnace, a cooling method of a ceramic fired body, and a method for manufacturing a honeycomb structured body.

### BACKGROUND ART

In recent years, particulates such as soot contained in exhaust gases that are discharged from internal combustion engines of vehicles, such as buses and trucks, and construction machines, have raised serious problems as contaminants harmful to the environment and the human body. There have been proposed various honeycomb filters using honeycomb structural bodies made from porous ceramic materials, which serve as filters that collect particulates in exhaust gases to purify the exhaust gases.

Conventionally, upon manufacturing such a honeycomb structured body, first, a wet mixture is prepared by mixing ceramic powder, a binder and a dispersant solution or the like with one another. Moreover, the wet mixture is continuously extrusion-molded through a die, and the extrusion-molded body is cut into a predetermined length. Thus, a rectangular pillar-shaped honeycomb molded body is manufactured.

Next, the resulting honeycomb molded body is dried, and predetermined cells are sealed, so that either one of ends of each cell is sealed by the plug material layer.

The honeycomb molded body thus sealed is carried in a degreasing furnace so that degreasing is carried out thereon.

Next, the resulting honeycomb molded body that has been degreased is put into a f iring furnace to carry out f iring thereon, and this is then cooled to manufacture a honeycomb structured body.

Thereafter, a sealing material paste is applied to the side faces of the honeycomb fired body, and the honeycomb fired bodies are mutually bonded, so that an aggregate of the honeycomb fired bodies in which a number of the honeycomb fired bodies are bound to one another by interposing the sealing material layers (adhesive layers) is manufactured. Next, the resulting aggregate of the honeycomb fired bodies is cut and machined into a predetermined shape, such as a cylindrical shape and a cylindroid shape, by using a cutting tool or the like, so that a honeycomb block is formed. Lastly, a sealing material paste is applied onto the periphery of the honeycomb block to form a sealing material layer (coat layer) ; thus, the manufacturing of the honeycomb structured body is completed. Such a honeycomb structural body is disclosed in US 4 364 760.

Here, in the present specification, in any of modes of the honeycomb molded body, the honeycomb fired body and the honeycomb structuredbody, among the faces forming the respective external shapes, those faces to which cells are exposed are referred to as end faces, and those faces other than the end faces are referred to as side faces.

### DISCLOSURE OF THE INVENTION PROBLEMS TO BE SOLVED BY THE INVENTION

Conventionally, since the cooling of the honeycomb structured bodies on which firing is carried out is conducted through natural radiation, a long period of time is required for the cooling of the honeycomb fired body to a necessary temperature, or the cooling tends to be adversely influenced by the external temperature. This inevitably causes a limitation in an attempt to improve the efficiency of the manufacturing of a honeycomb structured body.

### MEANS FOR SOLVING THE PROBLEMS

In order to solve the above-mentioned problems, the present inventors have intensively studied, and have found that by using a cooling apparatus having a plurality of blowers, the honeycomb fired body is efficiently cooled. Hence, a cooling apparatus for a firing body, a firing furnace and a cooling method of a ceramic fired body of the present invention, as well as a method for manufacturing a honeycomb structured body of the present invention that carries out a firing and a cooling by using such cooling apparatus and firing furnace, have been completed.

More specifically, a cooling apparatus for a fired body in accordance with a first aspect of the present invention is a cooling apparatus for a fired body, comprising: a transporting member for transporting a firing jig in which a ceramic fired body is housed; a plurality of blowers for cooling the ceramic fired body; and a suction mechanism for changing the atmosphere inside the firing jig from an inert gas atmosphere to an air atmosphere.

In the cooling apparatus for a fired body of the first aspect of the present invention, the plurality of blowers are desirably placed at both sides with respect to the transporting member. The suction mechanism is desirably placed at the upper side with respect to the transporting member. Moreover, the cooling apparatus for a fired body desirably further comprises
a removing member for removing deposits adhering to the firing jig.

The cooling apparatus for a fired body of the first aspect of the present invention is desirably installed in a firing furnace or next to a carrying-out port of the firing furnace.

A firing furnace in accordance with a second aspect of the present invention is a firing furnace comprising: a transporting member for transporting a firing jig in which a ceramic molded body is housed from a carrying-in port toward a carrying-out port; a heating unit for heating the ceramic molded body; and the cooling apparatus for a fired body of the first aspect of the present invention, the cooling apparatus disposed such that a distance between the cooling apparatus and the carrying-out port is smaller than a distance between the heating unit and the carrying-out port.

A cooling method of a ceramic fired body in accordance with a third aspect of the present invention is a cooling method of a ceramic fired body in which cooling is carried out by using a cooling apparatus comprising a transporting member for transporting a firing jig in which a ceramic fired body is housed, wherein the cooling apparatus further comprises a plurality of blowers, and ceramic fired body which is housed inside the firing jig placed on the transporting member is cooled by the blowers.

In the cooling method of a ceramic fired body of the third aspect of the present invention, the ceramic fired body is desirably cooled to 20 to 80°C in 30 to 120 minutes.

In the cooling method of a ceramic fired body of the third aspect of the present invention, the cooling apparatus desirably comprises a suction mechanism for sucking the internal area of the cooling apparatus. Further, the plurality of blowers are desirably placed at both sides with respect to the transporting member. Moreover, the suction mechanism is desirably placed at the upper side with respect to the transporting member.

In the cooling method of a ceramic fired body of the third aspect of the present invention, the cooling apparatus desirably further comprises a removing member for removing deposits adhering to the firing jig.

A method for manufacturing a honeycomb structured body in accordance with a fourth aspect of the present invention is a method for manufacturing a honeycomb structured body, comprising: manufacturing a pillar-shaped honeycomb molded body having a large number of cells longitudinally placed in parallel with one another with a cell wall therebetween, by molding a ceramic rawmaterial; firing the honeycombmoldedbody in a firing jig to manufacture a honeycomb structured body comprising a honeycomb firedbody, and further comprising: preparing a cooling apparatus comprising a transporting member for transporting the firing jig; and a plurality of blowers; and cooling the honeycomb fired body by using the cooling apparatus after the firing of the honeycomb molded body inside the firing jig.

In the method for manufacturing a honeycomb structured body of the fourth aspect of the present invention, the cooling desirably cools ceramic fired body 20 to 80°C in 30 to 120 minutes.

In the method for manufacturing a honeycomb structured body of the fourth aspect of the present invention, the cooling apparatus desirably comprises a suction mechanism for sucking the internal area of the cooling apparatus. Further, the plurality of blowers are desirably placed at both sides with respect to the transporting member. Moreover, the suction mechanism is desirably placed at the upper side with respect to the transporting member.

In the method for manufacturing a honeycomb structured body of the fourth aspect of the present invention, the cooling apparatus desirably further comprises a removing member for removing deposits adhering to the firing jig.

A method for manufacturing a honeycomb structured body in accordance with a fifth aspect of the present invention is a method for manufacturing a honeycomb structured body comprising: manufacturing a pillar-shaped honeycomb molded body having a large number of cells longitudinally placed in parallel with one another with a cell wall therebetween, by molding a ceramic rawmaterial; firing the honeycombmoldedbody in a firing jig by using a firing furnace to manufacture a honeycomb structured body comprising a honeycomb fired body; and further comprising: preparing a firing furnace comprises a cooling apparatus comprising a transporting member for transporting the firing jig; and a plurality of blowers; and firing the honeycomb molded body in the firing jig to manufacture the honeycomb fired body; and cooling of the honeycomb fired body, the firing and the cooling carried out in the firing furnace.

In the method for manufacturing a honeycomb structured body of the fifth aspect of the present invention, the cooling desirably cools ceramic fired body 20 to 80°C in 30 to 120 minutes.

In the method for manufacturing a honeycomb structured body of the fifth aspect of the present invention, the cooling apparatus desirably comprises a suction mechanism for sucking the internal area of the cooling apparatus. Further, the plurality of blowers are desirably placed at both sides with respect to the transporting member. Moreover, the suction mechanism is desirably placed at the upper side with respect to the transporting member.

In the method for manufacturing a honeycomb structured body of the fifth aspect of the present invention, the cooling apparatus desirably further comprises a removing member for removing deposits adhering to the firing jig.

### EFFECTS OF THE INVENTION

In the cooling apparatus for a fired body of the first aspect of the present invention, the ceramic fired body the temperature of which has been raised through the firing can be cooled in a short period of time without being influenced from the external temperature.
Moreover, since the ceramic fired body is cooled in its housed state inside the firing jig, the ceramic fired body is indirectly cooled without being directly exposed to a cooling air flow from the blowers. Consequently, despite the fact that the ceramic fired body is cooled in a shorter period of time in comparison with the conventional method, upon cooling the ceramic fired body, it becomes possible to prevent cracks and the like from occurring due to a thermal impact or the like.

In the firing furnace of the second aspect of the present invention, since the above-mentioned cooling apparatus of the present invention is installed therein, the ceramic molded body can be of course fired, and the resulting ceramic fired body can be efficiently cooled in a short period of time.

In the cooling method of a ceramic fired body of the third aspect of the present invention, since the ceramic fired body the temperature of which has been raised through the firing can be cooled by using a predetermined cooling apparatus, the period of time required for the cooling can be shortened and the ceramic molded body can be cooled efficiently without being influenced from the external temperature.
Moreover, since the ceramic fired body is cooled in its housed state inside the firing jig, the ceramic fired body is indirectly cooled without being directly exposed to a cooling air flow from the blowers. Consequently, despite the fact that the ceramic fired body is cooled in a shorter period of time in comparison with conventional method, upon cooling the ceramic fired body, it becomes possible to prevent cracks and the like from occurring due to a thermal impact or the like.

In the method for manufacturing a honeycomb structured body of the fourth aspect of the present invention, since the honeycomb fired body is cooled by using a predetermined cooling apparatus, the honeycomb fired body that has been fired and has a temperature rise can be cooled in a short period of time; therefore, it is possible to improve the production efficiency of the honeycomb structured body.
Moreover, upon cooling, the honeycomb fired body is indirectly cooled without being directly exposed to a cooling air flow from the blowers. Consequently, despite the fact that the honeycomb fired body is cooled in a shorter period of time in comparison with the conventional method, upon cooling the honeycomb fired body, it becomes possible to prevent cracks and the like from occurring due to a thermal impact or the like, and consequently to ensure the quality of the honeycomb structured body.

In the method for manufacturing a honeycomb structured body of the fifth aspect of the present invention, since the firing and the cooling are carried out by using a firing furnace provided with a predetermined cooling apparatus, the honeycomb fired body that has been fired and has a temperature rise can be cooled in a short period of time; therefore, it is possible to improve the production efficiency of the honeycomb structured body.
Moreover, during the cooling, the honeycomb fired body is indirectly cooled without being directly exposed to a cooling air flow from the blowers. Consequently, despite the fact that the honeycomb fired body is cooled in a shorter period of time in comparison with the conventional method, upon cooling the ceramic fired body, it becomes possible to prevent cracks and the like from occurring due to a thermal impact or the like, and consequently to ensure the quality of the honeycomb structured body.

### BEST MODE FOR CARRYING OUT THE INVENTION

First, referring to the drawings, the following description will discuss a cooling apparatus for a fired body in accordance with a first aspect of the present invention, a firing furnace in accordance with a second aspect of the present invention and a cooling method of a ceramic fired body in accordance with a third aspect of the present invention.
Here, in the first to third aspects of the present invention, a ceramic fired body to be cooled may be any fired body as long as it is obtained by firing a ceramic molded body. With respect to the ceramic fired body, for example, the honeycomb fired body and the like may be used.

A cooling apparatus for a fired body in accordance with the first aspect of the present invention includes: a transporting member for transporting a firing jig in which a ceramic fired body is housed; a plurality of blowers for cooling the ceramic fired body; and a suction mechanism for changing the atmosphere inside the firing jig from an inert gas atmosphere to an air atmosphere.

A firing furnace in accordance with the second aspect of the present invention includes: a transporting member for transporting a firing jig in which a ceramic molded body is housed from a carrying-in port toward a carrying-out port; a heating unit for heating the ceramic molded body; and the cooling apparatus for a fired body of the first aspect of the present invention, which is disposed such that a distance between the cooling apparatus and the carrying-out port is smaller than a distance between the heating unit and the carrying-out port.

A cooling method of a ceramic fired body in accordance with a third aspect of the present invention is a cooling method of a ceramic fired body in which cooling is carried out by using a cooling apparatus comprising a transporting member for transporting a firing jig in which a ceramic fired body is housed, wherein the cooling apparatus further comprises a plurality of blowers, and ceramic fired body which is housed inside the firing jig placed on the transporting member is cooled by the blowers.

Here, the firing furnace of the second aspect of the present invention is provided with the cooling apparatus for a fired body in accordance with the first aspect of the present invention. Moreover, the cooling method of a ceramic fired body of the third aspect is desirably carried out by using the cooling apparatus for a fired body in accordance with the first aspect of the present invention.
Therefore, the following description will first discuss the cooling apparatus for a fired body of the first aspect of the present invention, next discuss the firing furnace of the second aspect of the present invention that is provided with the cooling apparatus for a fired body, and then discuss the cooling method of the third aspect of the present invention.
Moreover, the first to third aspects of the present invention will be discussed by exemplifying a honeycomb fired body shown in Figs. 4 (a) and 4 (b) as the ceramic fired body to be cooled. Of course, the ceramic fired body to be cooled in the first to third aspects of the present invention is not limited to the honeycomb fired body, and various ceramic fired bodies may be used as the subject to be cooled.

Fig. 1 is a perspective view that schematically shows a cooling apparatus for a fired body in accordance with the first aspect of the present invention. As shown in Fig. 1, a cooling apparatus 30 for a fired body is provided with a transporting member 31 for transporting a firing jig 33 in which a honeycomb fired body 36 is housed, a plurality of blowers 32 that are placed at both sides with respect to the transporting member 31, and used for cooling the honeycomb fired body 36, and a suction mechanism 34, placed at the upper side with respect to the transporting member 31, which changes the atmosphere inside the firing jig 33 from an inert gas atmosphere to an air atmosphere. Here, a removing member 35, for removing deposits adhering to the firing jig 33 in a firing, is attached in a manner so as to enclose the firing jig 33 that has been transported.

With respect to the transporting member 31, not particularly limited as long as it allows the firing jig 33 to be smoothly transported, and for example, a conveyor, such as a belt conveyor and a chain conveyor, a transporting device of a walking beam type and the like may be used.

In the cooling apparatus 30 for a fired body, the honeycomb fired body 36 inside the firing jig 33 carried out from a firing furnace is transported by the transporting member 31 from a carrying-in port in its housed state inside the firing jig 33, and cooled by the blowers 32 placed at both sides with respect to the transporting member 31, and then carried out from a carrying-out port. In this case, the honeycomb fired body 36 is maintained in the housed state inside the firing jig 33, with the result that the honeycomb fired body 36 is not directly exposed to a cooling air flow from the blowers 32. In this manner, since the honeycomb fired body 36 is not locally cooled, it is possible to reduce a thermal impact or the like imposed on the honeycomb fired body 36, and consequently to prevent cracks and the like from occurring in the honeycomb fired body 36.
Here, for convenience of explanation, the honeycomb fired body 36 is illustrated in an exposed state in the firing jig 33 shown in Fig. 1; however, a roof plate is normally mounted on the uppermost portion of the firing jig 33, and the honeycomb fired body 36 is housed in the firing jig 33 in a non-exposed state.

Here, since the inside of the cooling apparatus 30 for a fired body is under a negative pressure (reduced pressure) by the suction mechanism 34, and is also kept in an air atmosphere, as will be described later, the honeycomb fired body 36 is cooled, and in the case where the atmosphere inside the firing jig 33 is an inert gas atmosphere, this inert gas atmosphere can be changed into an air atmosphere.

When the firing jig 33 has been transported to the position of the removing member 35 having a brush or the like, the brush or the like of the removing member 35 removes deposits adhering to the surface of the firing jig 33 through its reciprocating movements, rotation movements or the like. The deposits, thus removed by the removing member 35, are sucked by the suction mechanism 34 attached to a position closer to the carrying-out port than the position where the removing member 35 is installed, and collected outside the cooling apparatus 30 for a fired body together with the inert gas. Here, the attached position of the removing member 35 is not particularly limited, as will be described later.

Thereafter, the firing jig 33 from which the deposits have been removed is transported through a carrying-out port, and transported to the next process. At this time, since the honeycomb fired body 36 has been cooled to a temperature that is sufficiently low to allow the succeeding treatment or inspection, the honeycomb fired body 36 can be directly sent to the next process without the necessity of a waiting process; thus, it becomes possible to improve the working efficiency.

Here, the firing jig 33, which is used upon firing a honeycomb molded body (ceramic molded body), is a firing jig made from a ceramic material, which can be used in a superposed state with a number of stages. The firing jig 33 is provided with a vent portion at its one portion so as to allow ventilation between a space surrounded by the firing jig 33 and the outside, when superposed. Therefore, during the firing and the cooling, the firing igs 33, each housing a honeycomb molded body (ceramic molded body), are superposed in multiple stages, and firing is carried out thereon; thus, the resulting honeycomb fired body 36 can be cooled by the cooling apparatus 30 for a fired body.

With respect to the blower 32, its structure is not particularly limited as long as a convection of an atmospheric gas is raised inside the firing jig 33, and a structure in which an air blow is formed by rotating blades at high speeds or a structure in which a pressure is applied to the atmospheric gas to form an air blow may be used. Moreover, the blower 32 may send a cooling air flow having the same temperature as the temperature of the inside of the cooling apparatus 30 for a fired body, or a cooling air flow having a different temperature. The temperature of cooling air flows to be sent from the blowers 32 can be appropriately changed by taking into consideration the properties of the honeycomb firedbody 36, working efficiency and the like.

Here, the suction mechanism 34 is being operated during at least the time when cooling in which the honeycomb fired body 36 is cooled by operating the cooling apparatus 30 for a fired body is carried out, so that air, warmed up by the honeycomb fired body is continuously or regularly sucked. For this reason, it is possible to cool the honeycomb fired body quickly.
Moreover, by operating the suction mechanism 34, the atmosphere inside the firing jig 33 can be changed into an air atmosphere.
The atmosphere inside the firing furnace is normally substituted by an inert gas atmosphere so as to suppress undesired reactions upon firing the honeycomb molded body (ceramic molded body), and in addition to the substituted atmosphere inside the firing furnace, the inside of the firing jig 33 is of course substituted by an inert gas atmosphere. When, upon cooling, the inside of the firing jig 33 is in an inert gas atmosphere, the inert gas atmosphere inside the firing jig 33 can be changed into an air atmosphere by operating the suction mechanism 34.

Moreover, the cooling apparatus 30 for a fired body is provided with an air intake (not shown) for taking in clean air from outside, and capable of continuously taking in clean air such as filtered air. Therefore, the inside of the cooling apparatus 30 for a fired body is maintained in an air atmosphere.

In the cooling apparatus for a fired body in accordance with the first aspect of the present invention, the blowers are desirably placed at both sides with respect to the transporting member.
As shown in Fig. 1, in the case where the blowers 32 are placed at both sides with respect to the transporting member 31, since the cooling air flow is uniformly applied to the firing jig 33, the firing jig 33 can be cooled equally so that the honeycomb fired body 36 housed in the firing jig 33 can also be cooled uniformly.

In this case, with respect to the blowers 32 placed at one of the sides of the transporting member 31 and at the other side of the transporting member 31, the numbers thereof may be the same or different from each other, as long as the honeycomb fired body 36 can be uniformly cooled.
Moreover, the installation intervals of the blowers 32 may be equal to or different from each other; however, from the viewpoint of a uniform cooling for the firing jig 33 (honeycomb fired body 36), the equal installation interval is more desirable.

With respect to the relative positions between the blowers at one of the sides and those at the other side, those may be placed face to face with each other, or may be placed alternately, as long as the honeycomb fired body 36 can be uniformly cooled. From the viewpoint of the cooling efficiency, those are desirably placed alternately.

In the cooling apparatus for a fired body in accordance with the first aspect of the present invention, the suction mechanism is desirably placed at the upper side with respect to the transporting member.
When deposits, dusts and the like, removed by the removing member 35, are scattered by air directed from the blowers 32, this arrangement allows the deposits, dusts and the like to be properly sucked and externally discharged without again adhering to the transporting member 31 and the firing jig 33.
Moreover, when a plurality of blowers are placed at both sides with respect to the transporting member, air, sent from the blowers, is heated due to heat obtained upon cooling the firing jig, and directed upward. When the suction mechanism is placed at the upper side with respect to the transporting member, the air that has been heated and directed upward can be efficiently sucked so that an inert gas, deposits, dusts and the like are efficiently sucked. In this manner, the suction mechanism 34 is also allowed to function as a dust collector.

Specifications such as a suction pressure and shape of the suction mechanism 34 can be properly altered by taking into consideration the ventilation capability, installation spaces and the like required for exchanging atmospheric gases. With respect to the shape of the suction mechanism 34, as shown in Fig. 1, a shape in which a suction port is formed only on one portion of the upper face of the cooling apparatus 30 for a fired body may be used, or a flange shape in which the entire upper face serves as a suction port, with the diameter of the suction port being gradually narrowed, may be used.

The cooling apparatus for a fired body of the first aspect of the present invention is desirably provided with a removing member for removing deposits adhering to the firing jig, as indicated in the cooling apparatus 30 for a fired body shown in Fig. 1.
When a firing jig to which deposits have adhered during the firing, as it is, is used in a new firing, the honeycomb fired body (ceramic fired body) tends to be adversely affected due to evaporation or the like of the deposits; however, when the removing member 35 is prepared, the deposits adhering to the firing jig 33 can be removed so that even when the firing jig 33 is used in the next firing, no adverse effects are given to the firing of the honeycomb molded body (ceramic molded body) so that the firing jig 33 can be used repeatedly without the necessity of carrying out the removing of the deposits separately. Therefore, the firing jig can be used repeatedly without the necessity of overlapped maintenance.
Here, the number of the removing members 35 is not particularly limited as long as a sufficient space is available in the cooling apparatus 30 for a fired body, and can be determined on demand.

With respect to the removing member, not particularly limited as long as it can remove deposits adhering to the firing jig, a brush as shown in Fig. 1 may be used, or a curtain-shaped member may be used. Moreover, the removing member is desirably designed to be made in contact with the upper face and side faces of the firing jig as shown in Fig. 1; however, it may be designed to be made in contact with only the upper face or only the side faces of the firing jig.
With respect to the material for the removing member, examples thereof include: resin, cloth and leather.
Moreover, the removing member may be prepared as a fixed member as shown in Fig. 1, or may have a mode in which it is driven through vibration, reciprocating movement, rotating movement or the like to remove the deposits.

With respect to the installation position of the removing member 35, not particularly limited, it may be installed at a position closer to the carrying-in port than the position where the suction mechanism 34 is installed or, in contrast, may be installed at a position closer to the carrying-out port than the position where the suction mechanism 34 is installed.
Moreover, it may be installed right below the suction mechanism 34. In either of the cases, the deposits can be efficiently removed by the removing member 35.
The removing member is desirably attached to the vicinity of the suction mechanism. This arrangement allows the deposits removed by the removing member to be sucked without being scattered, making it possible to maintain the inside of the cooling apparatus for a fired body in a clean state.

The cooling apparatus for a fired body of the first aspect is desirably ins tailed next to the carrying-out port of the firing furnace. When the cooling apparatus for a fired body is installed next to the carrying-out port of the firing furnace, the honeycomb fired body (ceramic fired body) can be cooled efficiently.
Fig. 2 (a) is a cross-sectional view that shows a mode in which the cooling apparatus for a fired body of the first aspect of the present invention is installed next to the carrying-out port of the firing furnace.
In the mode shown in Fig. 2 (a), the cooling apparatus 30 for a fired body is installed next to a carrying-out port 10b of the firing furnace 10. Here, although omitted from the illustration, the firing furnace 10 is a continuous furnace, and the honeycomb molded body, transported through a carrying-in port 10a, is fired in the furnace, and then carried out through the carrying-out port 10b as a honeycomb fired body. The honeycomb fired body, thus transported through the carrying-out port 10b, is then successively transported into the cooling apparatus 30 for a fired body where it is cooled by the blowers 32 as described earlier.
Moreover, in the mode shown in Fig. 2(a), a continuous single transporting member 31 is used as a transporting member for transporting the honeycomb fired body through the cooling apparatus 30 for a fired body and as a transporting member for transporting the honeycomb molded body through the firing furnace 10; however, in this case, the transporting member is not necessarily prepared as the continuous single transporting member, and another structure may be used in which respectively different transporting members are used in the firing furnace and in the cooling apparatus for a fired body so that after the carrying-out from the firing furnace is carried out, the transporting members are switched to support the firing jig 33 before the carrying-in to the cooling apparatus for a fired body.
Moreover, the firing furnace next to which the cooling apparatus for a fired body is installed is not limited to a continuous furnace as shown in Fig. 2 (a), and may be prepared as a batch furnace.

Furthermore, the cooling apparatus for a fired body in accordance with the first aspect of the present invention is also desirably installed inside the firing furnace.
Fig. 2 (b) is a cross-sectional view that shows the firing furnace in which the cooling apparatus for a fired body of the first aspect of the present invention is installed.
When the cooling apparatus for a fired body is installed inside the firing furnace, the honeycomb fired body (ceramic fired body) can be cooled efficiently.
In addition, in the case where the cooling apparatus for a fired body is provided with the suction mechanism, since an inert gas atmosphere can be changed into an air atmosphere, the cooling apparatus for a fired body is allowed to function as both of a cooling unit and a degassing unit in the conventional firing furnace, thereby making it possible to save the space in the firing furnace and consequently to provide a further efficient method.

As shown in Fig. 2(b), from the carrying-in port 20a to the carrying-out port 20b inside the firing furnace 20, a degassing unit 21, a pre-heating unit 22, a heating unit 23, an cooling-down unit 24 and the cooling apparatus 40 for a fired body are successively installed.
Here, the structure of the cooling apparatus 40 for a fired body is the same as described earlier; therefore, the description thereof is omitted.

The heating unit 23 has a structure in which a cylinder-shapedmuffle 11 is formed so as to ensure a space through which the firing jig 33 housing the molded body therein passes. Here, heaters 12 are installed above and below the muffle 11 with predetermined intervals, and a heat-insulating layer 13 is formed in a manner so as to surround the muffle 11 and the heater 12. Moreover, a heat-insulating layer attaching member 16 for attaching the heat-insulating layer 13 is placed outside the heat-insulating layer 13, and a furnace-cooling member (water-cooling jacket) 14 is installed outside the heat-insulating layer attaching member 16, that is, on the outermost surface of the firing furnace 20.

The atmosphere inside the firing furnace 20 (inside of the pre-heating unit 22, the heating unit 23 and the cooling-down unit 24) is exchanged by an inert gas atmosphere by an inert gas 17 introduced from the outside, and isolated from the ambient atmosphere by the furnace cooling member 14. A cooling fluid, such as water, is allowed to flow the inside of the cooling furnace member 14 so that the cooling furnace member 14 is maintained at a predetermined temperature.
The atmosphere of the inside of the firing furnace 20 may be set to a predetermined atmosphere depending on the kind of a ceramic molded body.

In the firing furnace 20, the heaters 12 are installed above and below the muffle 11; however, the installation position of the heaters is not limited to this, and the heaters 12 may be installed at any place as long as they are on the peripheral portion of the muffle 11. The entire floor portion of the muffle 11 is supported by a supporting member, not shown, and the firing jig 33 housing the honeycomb molded body (ceramic molded body) therein is allowed to pass through it. The muffle 11 is placed over the entire portion of the firing furnace 20 except for the degassing unit 21 and the cooling apparatus 40 for a fired body.

Each heater 12 is a heat generating member made of graphite or the like, and the heater 12 is connected to a power supply (not shown) located outside through a terminal 18. The heaters 12 are installed in the heating unit 23, and are also installed in the pre-heating unit 22, if necessary.

The heat-insulating layers 13, which block heat generated from the heating unit 23 and heat transmitted from the heating unit 23, are placed on the pre-heating unit 22, the heating unit 23 and the cooling-down unit 24. In the heating unit 23, the heat-insulating layer 13 is placed so as to surround the heater 12, and the heat-insulating layer 13 is attached and secured to the heat-insulating layer attaching member 16 installed right outside thereof. Moreover, the cooling furnace member 14 is placed over the entire area except for the degassing unit 21 on the outermost side.

The degassing unit 21 is installed so as to change the atmosphere of the inside and peripheral portion of the firing jig 43 to be carried in into an inert gas atmosphere for use in firing. With respect to the sequence of processes for exchanging the atmosphere in the degassing unit 21, after the firing jig 33 mounted on the supporting base has been carried in, the degassing unit 21 is once evacuated, and an inert gas is then directed thereto so that the atmosphere of the inside and periphery of the firing jig 43 is changed into an inert gas atmosphere.

After the atmosphere inside the firing jig 43 has been changed by the degassing unit 21, the pre-heating unit 22 gradually raises the temperature of the firing jig 33 in which the honeycomb molded body (ceramic molded body) is housed by using the attached heaters, or by utilizing the heat of the heating unit.

Next, the firing jig 33 is transported to the heating unit 23 by the transporting means 19, and firing is carried out on the honeycomb molded body in the heating unit 23. Upon completion of the firing of the honeycomb molded body, the firing jig 43 after the firing is gradually cooled in the cooling-down unit 24.

The firing jig 43 is transported to the cooling apparatus 40 for a fired body installed inside the firing furnace 20 so that the temperature of the firing jig 43 is lowered to a predetermined temperature by using a plurality of blowers 32 installed in the cooling apparatus 40 for a fired body.

In the cooling apparatus 40 for a fired body, while the firing jig 43 is cooled to the predetermined temperature, deposits adhering to the firing jig 43 are removed by a removing member 35 installed on demand, and the atmosphere inside the firing jig 43 is exchanged from an inert gas atmosphere to an air atmosphere by using a suction mechanism (not shown) attached at the upper side with respect to the transporting means or the transporting member, and the firing jig 43 is carried out through the carrying-out port 20b; thus, the firing are completed.

Here, in the firing furnace 20, the cooling apparatus 40 for a fired body is disposed such that a distance between the cooling apparatus 40 for a fired body and the carrying-out port is smaller than a distance between the heating unit 23 and the carrying-out port. In the firing furnace 20, the cooling apparatus 40 for a fired body is placed at any position as long as it is located at least behind the heating unit 23, when viewed in the transporting direction of the transporting means 19.

In this manner, even in the case where the cooling apparatus 40 for a fired body is installed inside the firing furnace 20, since the suction mechanism for use in exchanging the atmosphere is prepared in the cooling apparatus 40 for a fired body, the atmosphere inside the firing jig 43 can be exchanged to an air atmosphere without the necessity of separately installing a degassing unit or the like in the firing furnace 20.

Moreover, in the case where the cooling apparatus 40 for a fired body is installed inside the firing furnace 20, in place of the transporting member 31 (see Fig. 1) forming the cooling apparatus 40 for a fired body, a transporting means 19 forming the firing furnace 20 may be extended into the cooling apparatus 40 for a fired body so that the firing jig 33 is transported, or the transporting member 31 and the transporting means 19 may be combined so as to carry out the transporting.

The above description has discussed in detail a mode in which the cooling apparatus for a fired body of the first aspect of the present invention is installed inside the firing furnace, and the firing furnace of this kind in which the cooling apparatus for a fired body is installed is also one aspect (firing furnace of the second aspect of the present invention) of the present invention.
In the firing furnace of the second aspect of the present invention, since no transporting of a honeycomb fired body (ceramic fired body) is separately prepared between the firing and the cooling of the honeycomb fired body (ceramic fired body), the firing and cooling can be continuously carried out so that the all the processes including the firing and the cooling can be efficiently carried out.

The following description will discuss a cooling method of a ceramic fired body in accordance with the third aspect of the present invention.
In the cooling method of a ceramic fired body of the third aspect of the present invention, a ceramic fired body, housed in a firing jig, is cooled by using a cooling apparatus provided with a plurality of blowers.

The cooling apparatus to be used in the cooling method of a ceramic f iredbody of the third aspect of the present invention is only required to include a transporting member and a plurality of blowers, and its structure is not particularly limited. With respect to the transporting member and the blowers, those transporting member and blowers used in the cooling apparatus for a fired body of the first aspect of the present invention are desirably used.
With respect to the cooling apparatus having such a structure, more specifically, a structure in which no suction mechanism is attached to the cooling apparatus for a fired body in accordance with the first aspect of the present invention that has been explained by reference to Fig. 1 is proposed. Of course, the cooling apparatus to be used in the cooling method of the third aspect of the present invention may be provided with a suction mechanism.
Since the structure of the above-mentioned cooling apparatus has been described in detail in the explanation of the cooling apparatus for a fired body, the description thereof is omitted, and the following description will mainly discuss cooling conditions and the like in accordance with the cooling method of the present invention.

In the cooling method of the third aspect of the present invention, the honeycomb fired body (ceramic fired body) is desirably cooled to 20 to 80°C in 30 to 120 minutes.
The temperature of the honeycomb fired body (ceramic fired body) that has been fired and transported through the cooling-down unit is about 280 to 300°C, and the cooling is carried out from this temperature range, under predetermined cooling conditions. In the case where the cooling time required to cool the honeycomb fired body (ceramic fired body) to 20°C becomes shorter than 30 minutes, the honeycomb fired body (ceramic fired body) fails to withstand a thermal impact caused upon cooling, resulting in damages such as cracks; in contrast, in the case where the cooling time required to cool to 80°C exceeds 120 minutes, it is considered that this operation is not effective from the viewpoint of improving the cooling efficiency. By adopting the above-mentioned cooling conditions, it becomes possible to efficiently cool the honeycomb fired body (ceramic fired body), while preventing the occurrence of cracks and the like.

In the third aspect of the present invention, the flow rate from the blowers installed in the cooling apparatus may be appropriately changed in accordance with the number of honeycomb fired bodies (ceramic fired bodies) to be cooled and the shape and the like of the firing jig, and, for example, the flow rate range from 10000 to 40000 m³/h can be adopted. With this flow rate range, it becomes possible to carry out an efficient cooling operation while preventing the occurrence of cracks or the like in the honeycomb fired body (ceramic fired body).

In the third aspect of the present invention, the temperature inside the cooling apparatus is desirably set in a range from 15 to 30°C. With this temperature range, it becomes possible to carry out an efficient cooling operation while preventing the occurrence of cracks or the like in the honeycomb fired body (ceramic fired body).

Moreover, the cooling apparatus to be used in the third aspect of the present invention is desirably provided with a suction mechanism for sucking the internal area of the cooling apparatus. With respect to this cooling apparatus provided with the suction mechanism, the cooling apparatus for a fired body in accordance with the first aspect of the present invention is desirably adopted.

The blowers are desirably placed at both sides with respect to the transporting member, and the cooling apparatus is also desirably provided with a removing member for removing deposits adhering to the firing jig. The reasons for these arrangements are the same as those explained in the cooling apparatus for a fired body of the first aspect of the present invention.

For example, in the case where the suction mechanism is made of a pillar-shaped pipe of 60 x 60 cm, although not particularly limited, the suction speed during the sucking by the suction mechanism is desirably set to 5 to 10 m/s inside the pipe. When the suction speed is set in the above-mentioned range, it is possible to efficiently exchange the atmosphere inside the firing jig and to effectively suck the exchanged inert gas and deposits.

With respect to the firing jig, the firing jig used in the cooling apparatus for a fired body of the first aspect of the present invention is desirably used. With respect to the number of stages of the superposed firing jigs, not particularly limited, one stage or a multiple superposed stages may be used. In particular, when 5 to 15 superposed stages are used, it becomes possible to improve the processing efficiency by using the multiple superposed stages, while preventing the cooling of the honeycomb fired body (ceramic fired body) from becoming insufficient.
Here, although not particularly limited, the number of honeycomb fired bodies (ceramic fired bodies) to be housed in one firing jig is desirably set to 7 to 20, when the cooling efficiency is taken into consideration.

As described above, in accordance with the cooling method for a ceramic fired body of the third aspect of the present invention, it becomes possible to efficiently carry out cooling, while preventing the occurrence of cracks and the like in a honeycomb fired body (ceramic fired body).

The following description will discuss a method for manufacturing a honeycomb structured body in accordance with a fourth aspect of the present invention.
A method for manufacturing a honeycomb structured body in accordance with a fourth aspect of the present invention is a method for manufacturing a honeycomb structured body, comprising: manufacturing a pillar-shaped honeycomb molded body having a large number of cells longitudinally placed in parallel with one another with a cell wall therebetween, by molding a ceramic raw material; firing the honeycomb molded body in a firing jig to manufacture a honeycomb structured body comprising a honeycombfiredbody, andfurthercomprising:preparingacooling apparatus comprising a transporting member for transporting the firing jig; and a plurality of blowers; and cooling the honeycomb fired body by using the cooling apparatus after the firing of the honeycomb molded body inside the firing jig.
In the present specification, the shape indicated by the word "pillar" refers to any desired shape of a pillar including a round pillar, an oval pillar, a polygonal pillar and the like.

The following description will discuss the method for manufacturing the honeycomb structured body of the fourth aspect of the present invention.

Fig. 3 is a perspective view that schematically shows one example of a honeycomb structured body in accordance with the present invention. Fig. 4(a) is a perspective view that schematically shows a honeycomb fired body forming the honeycomb structured body in accordance with the present invention. Fig. 4(b) is a cross-sectional view taken along line A-A.

In the honeycomb structured body 130, a plurality of honeycomb fired bodies 140 shown in Figs. 4 (a) and 4 (b) are bound to one another by interposing sealing material layers (adhesive layers) 131 to form a honeycomb block 133, and a sealing material layer (coat layer) 132 is further formed on the periphery of this honeycomb block 133.
Moreover, as shown in Figs. 4 (a) and 4 (b), the honeycomb fired body 140 has a large number of cells 141 longitudinally placed in parallel with one another, and each cell wall 143 that separates the cells 141 is allowed to function as a filter.

In other words, as shown in Fig. 4 (b), each of the cells 141, formed in the honeycomb fired body 140, is sealed with a plug material layer 142 at either one of ends on its exhaust gas inlet side and exhaust gas outlet side, so that exhaust gases that have entered one cell 141 are discharged from another cell 141 after having always passed through each cell wall 143 that separates the cells 141. When exhaust gases pass through the cell wall 143, particulates are captured by the cell wall 143, so that the exhaust gases are purified.

Here, the following description will discuss the method for manufacturing a honeycomb structured body in which powder of silicon carbide that is a ceramic raw material is used, by exemplifying manufacturing of a honeycomb structured body which is mainly composed of silicon carbide as a constituent material.
Of course, the main component of constituent materials for the honeycomb structured body is not intended to be limited by silicon carbide, and, other examples thereof include: nitride ceramic materials, such as aluminum nitride, silicon nitride, boron nitride and titanium nitride, carbide ceramic materials, such as zirconium carbide, titanium carbide, tantalum carbide and tungsten carbide, oxide ceramic materials, such as alumina, zirconia, cordierite, mullite, and aluminum titanate, and the like.
Among these, non-oxide ceramic materials are desirably used, and in particular, silicon carbide is more desirably used. Silicon carbide is used because of its superior heat resistant property, mechanical strength, thermal conductivity and the like. Here, materials, such as a silicon-containing ceramic material formed by blending metal silicon in the above-mentioned ceramic material and a ceramic material that is combined by silicon or a silicate compound, may also be used as the constituent materials, and among these, a material in which metal silicon is blended in silicon carbide (silicon-containing silicon carbide) is desirably used.

First, inorganic powder, such as silicon carbide powders having different average particle diameters, and an organic binder are dry-mixed to prepare mixed powder, and a liquid-state plasticizer, a lubricant and water are mixed to prepare a mixed liquid, and the mixed powder and the mixed liquid are mixed by using a wet-mixing device so that a wet mixture for use in manufacturing a molded body is prepared.

With respect to the particle diameter of silicon carbide powder, although not particularly limited, those which are less susceptible to shrinkage in the succeeding firing are desirably used, and for example, mixed powder, prepared by combining 100 parts by weight of powder having an average particle diameter from 0.3 to 50 µm with 5 to 65 parts by weight of powder having an average particle diameter from 0.1 to 1.0 µm, is desirably used.
In order to adjust the pore diameter and the like of the honeycomb fired body, it is necessary to adjust the firing temperature, and the pore diameter can be adjusted by adjusting the particle diameter of the inorganic powder.

With respect to the above-mentioned organic binder, not particularly limited, examples thereof include: methylcellulose, carboxy methylcellulose, hydroxy ethylcellulose, polyethylene glycol and the like. Among these, methylcellulose is more desirably used.
In general, the compounding amount of the above-mentioned binder is desirably set to 1 to 10 parts by weight with respect to 100 parts by weight of the inorganic powder.

With respect to the above-mentioned plasticizer, not particularly limited, for example, glycerin and the like may be used.
Moreover, with respect to the lubricant, not particularly limited, for example, polyoxy alkylene-based compounds, such as polyoxyethylene alkyl ether and polyoxy propylene alkyl ether and the like may be used.
Specific examples of the lubricant include: polyoxyethylene monobutyl ether and polyoxypropylene monobutyl ether.
Here, the plasticizer and the lubricant are not necessarily contained in the mixed material powder depending on cases.

Upon preparing the wet mixture, a dispersant solution may be used, and with respect to the dispersant solution, examples thereof include: water, alcohol such as methanol, an organic solvent such as benzene, and the like.
Moreover, a molding auxiliary may be added to the wet mixture.
With respect to the molding auxiliary, not particularly limited, examples thereof include: ethylene glycol, dextrin, fatty acid, fatty acid soap, polyalcohol and the like.

Furthermore, a pore forming agent, such as balloons that are fine hollow spheres composed of oxide-based ceramics, spherical acrylic particles, graphite and the like may be added to the above-mentioned wet mixture, if necessary.
With respect to the above-mentioned balloons, not particularly limited, for example, alumina balloons, glass micro-balloons, shirasu balloons, fly ash balloons (FA balloons), mullite balloons and the like may be used. Among these, alumina balloons are more desirably used.

Here, with respect to the wet mixture using silicon carbide powder, prepared as described above, the temperature thereof is desirably set to 28°C or less. When the temperature is too high, the organic binder tends to be gelatinized.
Moreover, the rate of organic components in the wet mixture is desirably set to 10% by weight or less, and the content of moisture is desirably set from 8.0 to 20.0% by weight or less.

Thewetmixture, thus prepared, is transported, and charged into a molding machine.
The wet mixture transported by the transporting device and charged into the molding machine is then extrusion-molded into a honeycomb molded body having a predetermined shape.
Next, the resulting honeycomb molded body is dried by using a drying apparatus, such as a microwave drying apparatus, a hot-air drying apparatus, a dielectric drying apparatus, a reduced-pressure drying apparatus, a vacuum drying apparatus, a frozen drying apparatus and the like so that a dried honeycomb molded body is formed.

Here, cutting is carried out on the honeycomb molded body thus formed, by using a cutting machine to cut the two ends thereof so that a honeycomb molded body having a predetermined length is formed.

Next, a predetermined amount of plug material paste that forms plugs is filled into ends on the outlet side of a group of cells on the inlet side and ends on the inlet side of a group of cells on the outlet side, if necessary, so that predetermined cells are sealed. Upon sealing the cells, a mask for sealing the cells is made in contact with the end face (that is, the cut face after the cutting) of the honeycomb molded body so that only the cells to be sealed are filled with the plug material paste.

With respect to the plug material paste, although not particularly limited, those plug material pastes that allow the plugs manufactured through post processes to have a porosity in a range from 30 to 75% are desirably used, and, for example, the same material as that of the wet mixture may be used.

The filling of the plug material paste can be carried out on demand, and when the plug material paste has been filled thereto, for example, the resulting honeycomb structured body obtained through the post process is desirably used as a honeycomb filter, and in the case where no plug material paste has been filled thereto, for example, the honeycomb structured body obtained through the post process is desirably used as a catalyst supporting body.

Next, the honeycomb molded body, which has the plug material paste filled therein, is transported to a degreasing furnace by using a degreasing furnace carrying-in device so as to be degreased.
The honeycomb molded body is carried in into the degreasing furnace by using the degreasing furnace carrying-in device face, and degreased under predetermined conditions (for example, 200 to 500°C).

Next, the honeycomb molded body on which degreasing has been carried out is fired in a firing jig, and the resulting honeycomb fired body is cooled by using a cooling apparatus in which a transporting member for transporting the firing jig and a plurality of blowers so that it is possible to manufacture a honeycomb fired body (see Figs. 4(a) and 4(b)) formed by a single fired body as a whole in which: a plurality of cells are longitudinally placed in parallel with one another with a cell wall therebetween, and either one of ends of the cells is sealed.

In the firing for the honeycomb molded body, the honeycomb molded body is housed in a firing jig, and firing thereof is carried out in this state. With respect to the firing jig, the firing jig, explained in the cooling apparatus for a fired body of the first aspect of the present invention, is desirably used.
Here, with respect to the firing conditions for the honeycomb molded body, those conditions conventionally used upon manufacturing a filter made from a porous ceramic material (for example, 1400 to 2300°C for 1 to 10 hours) may be used.

Thereafter, the resulting honeycomb fired body is cooled in a fired body cooling in which a cooling apparatus provided with a transporting member for transporting the firing jig and a plurality of blowers is used. With respect to the cooling method in the present fired body cooling, the cooling method, explained in the cooling method for the ceramic fired body of the third aspect of the present invention, is desirably used.

Moreover, the cooling desirably cools ceramic fired body 20 to 80°C in 30 to 120 minutes.

Furthermore, the cooling apparatus is desirably provided with a suction mechanism for sucking the internal area of the cooling apparatus, the plurality of blowers are desirably placed at both sides with respect to the transporting member, and the suction mechanism is desirably placed at the upper side with respect to the transporting member.
The cooling apparatus is desirably provided with a removing member for removing deposits adhering to the firing jig.
In the fired body cooling relating to the method for manufacturing a honeycomb structured body in accordance with the fourth aspect of the present invention, the reasons for the above-mentioned arrangements to be desirably used have been explained in the cooling method of a ceramic fired body in accordance with the third aspect of the present invention; therefore, the description thereof is omitted.

Next, a sealing material paste to form a sealing material layer (adhesive layer) is applied onto side faces of the honeycomb fired body thus cooled with an even thickness to form a sealing material paste layer, and laminating for forming another honeycomb fired body on this sealing material paste layer is successively repeated so that an aggregate of honeycomb fired bodies having a predetermined size is manufactured.

With respect to the sealing material paste, examples thereof include an inorganic binder, an organic binder and a material made from inorganic fibers and/or inorganic particles.
With respect to the inorganic binder, for example, silica sol, alumina sol and the like may be used. Each of these may be used alone or two or more kinds of these may be used in combination. Among the inorganic binders, silica sol is more desirably used.

With respect to the organic binder, examples thereof include polyvinyl alcohol, methyl cellulose, ethyl cellulose, carboxymethyl cellulose, and the like. Each of these may be used alone or two or more kinds of these may be used in combination. Among the organic binders, carboxymethyl cellulose is more desirably used.

With respect to the inorganic fibers, examples thereof include ceramic fibers, such as silica-alumina, mullite, alumina, silica, and the like. Each of these may be used alone or two or more kinds of these may be used in combination. Among the inorganic fibers, alumina fibers are more desirably used.

With respect to the inorganic particles, examples thereof include carbides and nitrides, and specific examples include inorganic powder or the like made from silicon carbide, silicon nitride and boron nitride. Each of these may be used alone, or two or more kinds of these may be used in combination. Among the inorganic particles, silicon carbide having superior thermal conductivity is desirably used.

Moreover, a pore forming agent, such as balloons that are fine hollow spheres composed of oxide-based ceramics, spherical acrylic particles, graphite and the like may be added to the above-mentioned sealing material paste, if necessary.
With respect to the above-mentioned balloons, not particularly limited, for example, alumina balloons, glass micro-balloons, shirasuballoons, flyashballoons (FAballoons), mullite balloons and the like may be used. Among these, alumina balloons are more desirably used.

Next, this aggregate of honeycomb fired bodies is heated so that the sealing material paste layers are dried and solidified to form sealing material layers (adhesive layers).
Next, cutting is carried out on the aggregate of honeycomb fired bodies in which a plurality of honeycomb fired bodies have been bonded to one another by interposing sealing material layers (adhesive layers), by using a diamond cutter or the like so that a cylindrical honeycomb block is manufactured.

Then, a sealing material layer (coat layer) is formed on the peripheral portion of the honeycomb block by using the above-mentioned sealing material paste so that a honeycomb structured body in which a sealing material layer (coat layer) is formed on the periphery of a cylindrical honeycomb block having a structure in which a plurality of honeycomb fired bodies are bound to one another by interposing sealing material layers (adhesive layers) is manufactured.

Thereafter, a catalyst is supported on the honeycomb structured body on demand. The supporting of the catalyst may be carried out on the honeycomb fired bodies prior to being formed into an aggregate.
In the case where a catalyst is supported thereon, an alumina film having a high specific surface area is desirably formed on the surface of the honeycomb structured body, and a co-catalyst and a catalyst such as platinum are applied onto the surface of the alumina film.

With respect to the method for forming the alumina film on the surface of the honeycomb structured body, for example, a method in which the honeycomb structured body is impregnated with a solution of a metal compound containing aluminum such as Al (NO₃) and then heated and a method in which the honeycomb structured body is impregnated with a solution containing alumina powder and then heated, are proposed.
With respect to the method for applying a co-catalyst to the alumina film, for example, a method in which the honeycomb structured body is impregnated with a solution of a metal compound containing a rare-earth element, such as Ce (NO₃)₃, and then heated is proposed.
With respect to the method for applying a catalyst to the alumina film, for example, a method in which the honeycomb structured body is impregnated with a solution of diammine dinitro platinum nitric acid ([Pt(NH₃)₂(NO₂)₂]HNO₃, platinum concentration: 4.53% by weight) and then heated is proposed.
Moreover, a catalyst may be applied through a method in which after the catalyst has been preliminarily applied to alumina particles, the honeycomb structured body is impregnated with a solution containing the alumina powder bearing the catalyst applied thereto, and then heated.

Here, the above-mentioned method for manufacturing a honeycomb structured body relates to an aggregated honeycomb structured body having a structure in which a plurality of honeycomb fired bodies are bound to one another by interposing sealing material layers (adhesive layers); however, the honeycomb structured body to be manufactured by the method of the present invention may be an integral honeycomb structured body in which a pillar-shaped honeycomb block is constituted by one honeycomb fired body. Here, desirably, the integral honeycomb structured body is mainly composed of a material such as cordierite and aluminum titanate.

Upon manufacturing such an integral honeycomb structured body, first, a honeycomb molded body of this kind is formed by using the same method as the method for manufacturing an aggregated honeycomb structured body except that the size of a honeycomb molded body to be molded through the extrusion-molding is greater than that of the aggregated honeycomb structured body.

Next, in the same manner as the method for manufacturing the aggregated honeycomb structured body, the honeycomb molded body is dried by using a drying apparatus, such as a microwave drying apparatus, a hot-air drying apparatus, a dielectric drying apparatus, a reduced-pressure drying apparatus, a vacuum drying apparatus, a frozen drying apparatus and the like.
Next, cutting is carried out on the dried honeycomb molded body, by using a cutting machine to cut the two ends thereof.

Next, a predetermined amount of plug material paste that forms plugs is filled into ends on the outlet side of a group of cells on the inlet side and ends on the inlet side of a group of cells on the outlet side so that predetermined cells are sealed.
Thereafter, in the same manner as the manufacturing method for the aggregated honeycomb structured body, the degreasing and firing are carried out to manufacture a honeycomb block, and by forming a sealingmaterial layer (coat layer), if necessary, an integral honeycomb structured body can be manufactured. Moreover, a catalyst may also be supported on the integral honeycomb structured body by using the same method.

With respect to the honeycomb structured body, the foregoing explanation has been given mainly on a honeycomb filter that is used to collect particulates in exhaust gases; however, the honeycomb structured body may also be desirably used as a catalyst supporting body (honeycomb catalyst) that converts exhaust gases.

In the method for manufacturing a honeycomb structured body of the fourth aspect of the present invention as explained above, it is possible to manufacture a honeycomb structured body by using highly efficient operations.
Moreover, upon manufacturing a honeycomb structured body through the above-mentioned method, since the cooling of the honeycomb fired body, which has been conventionally carried out through natural radiation, is carried out by using a predetermined cooling apparatus, a sequence of working can be carried out continuously in a more effective manner. Therefore, the method for manufacturing a honeycomb structured body in the fourth aspect of the present invention can also improve the efficiency of the all manufacturing method.

The following description will discuss a method for manufacturing a honeycomb structured body in accordance with the fifth aspect of the present invention.
A method for manufacturing a honeycomb structured body in accordance with a fifth aspect of the present invention is a method for manufacturing a honeycomb structured body comprising: manufacturing a pillar-shapedhoneycombmoldedbody having a large number of cells longitudinally placed in parallel with one another with a cell wall therebetween, by molding a ceramic rawmaterial; firing the honeycomb molded body in a firing jig by using a firing furnace to manufacture a honeycomb structured body comprising a honeycomb fired body; and further comprising: preparing a firing furnace comprises a cooling apparatus comprising a transporting member for transporting the firing jig; and a plurality of blowers; and firing the honeycomb molded body in the firing jig to manufacture the honeycomb fired body; and cooling of the honeycomb fired body, the firing and the cooling carried out in the firing furnace.
In the method for manufacturing a honeycomb structured body of the fifth aspect of the present invention, the same method as the method for manufacturing a honeycomb structured body in accordance with the fourth aspect of the present invention can be used except for the firing and the cooling; therefore, with respect to the method for manufacturing a honeycomb structured body of the fifth aspect of the present invention, the following description will mainly discuss the firing and the cooling.

In the method for manufacturing a honeycomb structured body in accordance with the fifth aspect of the present invention, first, a honeycomb molded body in which either one of ends of the cells is sealed with a plug material paste on demand is formed by using the same method as the method for manufacturing a honeycomb structured body of the fourth aspect of the present invention, and degreasing is carried out on the honeycomb molded body.

Next, a firing in which the honeycomb molded body is fired in the firing jig by using the firing furnace in which the transporting member for transporting the firing jig and the plurality of blowers are installed to form a honeycomb fired body and the cooling in which the honeycomb fired body is cooled are carried out. More specifically, the above-mentioned firing and cooling are desirably carried out by using the firing furnace in accordance with the second aspect of the present invention.

With respect to the firing conditions, in the same manner as the method for manufacturing a honeycomb structured body of the fourth aspect of the present invention, those conditions conventionally used upon manufacturing a filter made from a porous ceramic material (for example, 1400 to 2300°C for 1 to 10 hours) may be used.
Moreover, in the above-mentioned cooling, the cooling desirably cools ceramic fired body 20 to 80°C in 30 to 120 minutes .
The reasons for the above-mentioned arrangements to be desirably used have been explained in the cooling method of a ceramic fired body in accordance with the third aspect of the present invention; therefore, the description thereof is omitted.

Furthermore, in the fifth aspect of the present invention, the cooling apparatus is desirably provided with a suction mechanism for sucking the internal area of cooling apparatus, the plurality of blowers are desirably placed at both sides with respect to the transporting member, and the suction mechanism is desirably placed at the upper side with respect to the transporting member.
The cooling apparatus is desirably provided with a removing member for removing deposits adhering to the firing jig.

After the honeycomb molded body has been fired and formed into a honeycomb fired body cooled to a predetermined temperature, an aggregate of the honeycomb fired bodies is formed and a honeycomb block is then manufactured by using the same manufacturing method as the honeycomb structured body of the fourth aspect of the present invention so that a honeycomb structured body is manufactured by further forming a sealing material layer (coat layer) thereon.
In the method for manufacturing the honeycomb structured body in accordance with the fifth aspect of the present invention also, a catalyst may be supported on a honeycomb structured body, if necessary, in the same manner as the method for manufacturing the honeycomb structured body in accordance with the fourth aspect of the present invention.

In the method for manufacturing the honeycomb structured body of the fifth aspect of the present invention also, an integral honeycomb molded body is formed by using the same method as method for manufacturing the honeycomb structured body of the fourth aspect of the present invention, that is, the method for manufacturing an aggregated honeycomb structured body, except that the size of a honeycomb molded body to be molded through extrusion-molding is greater than that of the aggregated honeycomb structured body.

With respect to the honeycomb structured body, the foregoing explanation has been given mainly on a honeycomb filter that is used to collect particulates in exhaust gases; however, the honeycomb structured body may also be desirably used as a catalyst supporting body (honeycomb catalyst) that converts exhaust gases.

In the method for manufacturing a honeycomb structured body of the fifth aspect of the present invention as explained above, it is possible to manufacture a honeycomb structured body by using highly efficient operations.
Moreover, upon manufacturing a honeycomb structured body through the above-mentioned method, since the firing and the cooling are carried out in the single firing furnace, a sequence of working can be carried out continuously in a more effective manner. Therefore, the method for manufacturing a honeycomb structured body in the fifth aspect of the present invention can also improve the efficiency of the entire manufacturing method.

### EXAMPLES

By way of specific examples, the present invention will be explained hereinafter in detail. However, the present invention is not limited only by these examples.
In these examples, upon manufacturing honeycomb fired bodies, the honeycomb fired bodies were cooled under various cooling conditions so that the time required for cooling and changes in the honeycomb fired body after the cooling were examined.

### (Example 1)

Powder of α-type silicon carbide having an average particle diameter of 10 µm (250 kg), powder of α-type silicon carbide having an average particle diameter of 0.5 µm (100 kg) and an organic binder (methylcellulose) (20 kg) were mixed to prepare mixed powder.
Next, separately, a lubricant (Uniloop, made by NOF Corporation) (12 kg), a plasticizer (glycerin) (5 kg) and water (65 kg) were mixed to prepare a liquid mixture, and this liquid mixture and the mixed powder were mixed by using a wet-type mixing machine so that a wet mixture was prepared.
The moisture content of the wet mixture thus prepared was 14% by weight.

Next, this wet mixture was transported to an extrusion molding machine by using a transporting device, and charged into a material charging port of the extrusion molding machine.
Here, the moisture content of the wet mixture immediately before the charging into the extrusion molding machine was 13.5% by weight.
The wet mixture was then extrusion-molded into a rawmolded body having a shape shown in Figs. 4 (a) and 4 (b), and not having its end portions sealed.

Next, after the raw molded body had been dried by using a microwave drying apparatus or the like, a plug material paste having the same composition as the wet mixture was filled into predetermined cells.
The honeycomb molded body to which the plug material paste had been filled was again dried by using a drying apparatus, and the honeycomb molded body thus dried was carried in a degreasing furnace. The honeycomb molded body, carried in the degreasing furnace, was degreased at 400°C.

Thereafter, by using the firing furnace 20 (continuous firing furnace) of the second aspect of the present invention shown in Fig. 2 (b), in a firing process, firing was carried out on the degreased honeycomb molded body, and the resulting honeycomb fired body was cooled in the cooling process.

More specifically, the honeycomb molded body, mounted on the firing jig, was put into a continuous firing furnace where it was fired at 2200°C in a normal-pressure argon atmosphere serving as an inactive gas for 3 hours.

Successively, a cooling apparatus 30 for a fired body having a structure shown in Fig. 1 was placed next to the carrying-out port of the continuous firing furnace, and cooling was carried out on the honeycomb fired body under conditions as shown in Table 1.

After the cooling, the honeycomb fired body, which was a silicon carbide sintered body, had a porosity of 40%, an average pore diameter of 12.5 µm, a size of 34.3 mm x 34.3 mm x 150 mm, the number of cells (cell density) of 46.5/cm² and a thickness of each cell wall of 0.20 mm.

### (Examples 2 to 5)

The same processes as Example 1 were carried out except that the cooling conditions in the cooling process were set to values shown in Table 1 to manufacture a honeycomb fired body.

### (Reference Examples 1 and 2)

The same processes as Example 1 were carried out except that the cooling conditions in the cooling process were set to values shown in Table 1 to carry out a swift cooling treatment so that a honeycomb fired body was manufactured.

### (Comparative Example 1)

The same processes as Example 1 were carried out except that the cooling process was carried out through natural radiation, without carrying out the cooling process by the cooling apparatus for a fired body.

### (Observation on state of honeycomb fired body)

### Breaking test

Referring to JIS R 1601, four-points bending tests were carried out under conditions of an upper-face span-to-span distance of 20 mm, a lower-face span-to-span distance of 133 mm, a speed of 10 mm/min and an applied load of 2940 N(300 kgf) by using an Instron 5582 so that the honeycomb fired body was observed as to whether or not there were any damages. Here, the number of the test pieces was set to ten.
The results are as shown in Table 1. Here, the applied load is an experience value of which a normal honeycomb fired body is not destroyed but a honeycomb fired body having defects such as cracks and the like is destroyed.

**Table 1**

| | Number of blowers (one side) | Number of blowers (total) | Flow rate of blowers [m³/h] | Speed of conveyor [m/min] | Cooling time [min] | Temperature after cooling [min] | Presence or absence of fracture upon breaking test |
|---|---|---|---|---|---|---|---|
| Example 1 | 3 | 6 | 30000 | 0.2 | 60 | 40 | Not present |
| Example 2 | 3 | 6 | 40000 | 0.2 | 60 | 30 | Not present |
| Example 3 | 3 | 6 | 35000 | 0.3 | 40 | 40 | Not present |
| Example 4 | 3 | 6 | 20000 | 0.15 | 80 | 40 | Not present |
| Example 5 | 3 | 6 | 10000 | 0.12 | 100 | 40 | Not present |
| Reference Example 1 | 3 | 6 | 50000 | 0.4 | 30 | 30 | Present |
| Reference Example 2 | 3 | 6 | 50000 | 0.48 | 25 | 40 | Present |
| Comparative Example 1 | Natural radiation | | | | 150 | 40 | Not present |

As clearly indicated by the results shown in Table 1, under the cooling conditions in Examples 1 to 5, the honeycomb fired body can be cooled to 30 to 40°C in 40 to 100 minutes and the cooled honeycomb fired body was not broken even under the breaking test; thus, it can be said that an efficient cooling was carried out under the cooling conditions in Examples 1 to 5.

In contrast, in the case of the honeycomb fired body in Comparative Example 1, although the state of the honeycomb fired body after the cooling was desirable without any fracture in the breaking test, it took 150 min to cool the honeycomb fired body to the same temperature as Example 1, resulting in the necessity of a cooling time of a great degree in comparison with the examples.

Moreover, in the case of Reference Examples 1 and 2, although the honeycomb fired body was cooled to 30 to 40°C in a short period of time such as 25 to 30 minutes, the honeycomb fired bodies were partially damaged at the time of the breaking test. Presumably, this is because of an influence of a thermal impact due to the swift cooling.

### BRIEF DESCRIPTION OF THE DRAWINGS

Fig. 1 is a perspective view that schematically shows a cooling apparatus for a fired body in accordance with the first aspect of the present invention.
Fig. 2 (a) is a cross-sectional view that shows a mode in which the cooling apparatus for a fired body of the first aspect of the present invention is placed next to the carrying-out port of a firing furnace.
Fig. 2(b) is a cross-sectional view that shows a firing furnace in which the cooling apparatus for a fired body of the first aspect of the present invention is placed.
Fig. 3 is a perspective view that schematically shows one example of a honeycomb structured body in accordance with the present invention.
Fig. 4 (a) is a perspective view that schematically shows a honeycomb fired body that forms one component of the honeycomb structured body in accordance with the present invention.
Fig. 4 (b) is a cross-sectional view taken along line A-A of Fig. 4(a).

### EXPLANATION OF SYMBOLS

- 10,: 20 Firing furnace
- 11: Muffle
- 12: Heater
- 13: Heat-insulating layer
- 14: Furnace-cooling member
- 16: Heat-insulating layer attaching member
- 17: Inert gas
- 19: Transporting means
- 21: Degassing unit
- 22: Pre-heating unit
- 23: Heating unit
- 24: Cooling-down unit
- 30,: 40 Cooling apparatus for fired body
- 31: Transporting member
- 32: Blower
- 33,: 34 Firing jig
- 35: Removing member
- 36: Honeycomb fired body

## Claims

1. A cooling apparatus for a fired body, comprising:
a transporting member for transporting a firing jig in which a ceramic fired body is housed;
a plurality of blowers for cooling said ceramic fired body; and
a suction mechanism for changing the atmosphere inside said firing jig from an inert gas atmosphere to an air atmosphere.

2. The cooling apparatus for a fired body according to claim 1,
wherein
said plurality of blowers are placed at both sides with respect to said transporting member.

3. The cooling apparatus for a fired body according to claim 1 or 2,
wherein
said suction mechanism is placed at the upper side with respect to said transporting member.

4. The cooling apparatus for a fired body according to any of claims 1 to 3,
further comprising:
a removing member for removing deposits adhering to said firing jig.

5. The cooling apparatus for a fired body according to any of claims 1 to 4,
which is installed in a firing furnace or next to a carrying-out port of the firing furnace.

6. A firing furnace comprising:
a transporting member for transporting a firing jig in which a ceramic molded body is housed from a carrying-in port toward a carrying-out port;
a heating unit for heating said ceramic molded body; and
the cooling apparatus for a fired body disclosed in any of claims 1 to 4,
said cooling apparatus disposed such that a distance between said cooling apparatus and said carrying-out port is smaller than a distance between said heating unit and said carrying-out port.

7. A cooling method of a ceramic fired body in which cooling is carried out by using a cooling apparatus comprising a transporting member for transporting a firing jig in which a ceramic fired body is housed,
wherein
said cooling apparatus further comprises a plurality of blowers, and
ceramic fired body which is housed inside the firing jig placed on said transporting member is cooled by said blowers.

8. The cooling method of a ceramic fired body according to claim 7,
wherein
said ceramic fired body is cooled to 20 to 80°C in 30 to 120 minutes.

9. The cooling method of a ceramic fired body according to claim 7 or 8,
wherein
said cooling apparatus comprises a suction mechanism for sucking the internal area of the cooling apparatus.

10. The cooling method of a ceramic fired body according to any of claims 7 to 9,
wherein
said plurality of blowers are placed at both sides with respect to said transporting member.

11. The cooling method of a ceramic fired body according to claim 9 or 10,
wherein
said suction mechanism is placed at the upper side with respect to said transporting member.

12. The cooling method of a ceramic fired body according to any of claims 9 to 11,
wherein
said cooling apparatus further comprises a removing member for removing deposits adhering to said firing jig.

13. A method for manufacturing a honeycomb structured body, comprising:
manufacturing a pillar-shaped honeycomb molded body having a large number of cells longitudinally placed in parallel with one another with a cell wall therebetween, by molding a ceramic raw material;
firing said honeycomb molded body in a firing jig to manufacture a honeycomb structured body comprising a honeycomb fired body, and
further comprising:
preparing a cooling apparatus comprising
a transporting member for transporting said firing jig; and
a plurality of blowers; and
cooling the honeycomb fired body by using said cooling apparatus after said firing of said honeycomb molded body inside the firing jig.

14. The method for manufacturing a honeycomb structured body according to claim 13,
wherein
said honeycomb molded body is fired and cooled in a firing jig by using a firing furnace comprising the cooling apparatus.

15. The method for manufacturing a honeycomb structured body according to claim 13 or 14,
wherein
said cooling cools ceramic fired body 20 to 80°C in 30 to 120 minutes.

16. The method for manufacturing a honeycomb structured body according to any of claims 13 to 15,
wherein
said cooling apparatus comprises a suction mechanism for sucking the internal area of the cooling apparatus.

17. The method for manufacturing a honeycomb structured body according to any of claims 13 to 16,
wherein
said plurality of blowers are placed at both sides with respect to said transporting member.

18. The method for manufacturing a honeycomb structured body according to any of claims 13 to 17,
wherein
said suction mechanism is placed at the upper side with respect to said transporting member.

19. The manufacturing method for a honeycomb structured body according to any of claims 13 to 18,
wherein
said cooling apparatus further comprises a removing member for removing deposits adhering to said firing jig.

## Patentansprüche

1. Kühlvorrichtung für einen erhitzten Körper, die umfasst:
ein Transportelement zum Transportieren einer Heizeinrichtung, in der ein erhitzter Keramikkörper aufgenommen ist;
eine Vielzahl von Gebläsen zum Kühlen des erhitzten Keramikkörpers; und
einen Saugmechanismus zum Ändern der Atmosphäre in der Heizeinrichtung von einer Inertgasatmosphäre in eine Luftatmosphäre.

2. Kühlvorrichtung für einen erhitzten Körper nach Anspruch 1, bei dem
die Vielzahl der Gebläse an beiden Seiten bezüglich des Transportelements angeordnet sind.

3. Kühlvorrichtung für einen erhitzten Körper nach Anspruch 1 oder 2, bei dem
der Saugmechanismus an der oberen Seite bezüglich des Transportmechanismus angeordnet ist.

4. Kühlvorrichtung für einen erhitzten Körper nach einem der Ansprüche 1 bis 3, ferner umfassend:
ein Entfernungselement zum Entfernen von Ablagerungen, die an der Heizeinrichtung anhaften.

5. Kühlvorrichtung für einen erhitzten Körper nach einem der Ansprüche 1 bis 4,
die in einem Heizofen oder in der Nähe zu einem Herausgabeanschluss des Heizofens installiert ist.

6. Heizofen, der umfasst:
ein Transportelement zum Transportieren einer Heizeinrichtung, in der ein geformter Keramikkörper aufgenommen ist, von einem Einbringanschluss zu einem Herausgabeanschluss;
eine Heizeinheit zum Erhitzen des geformten Keramikkörpers; und
die Kühlvorrichtung für einen erhitzten Körper, die in einem der Ansprüche 1 bis 4 offenbart ist,
wobei die Kühlvorrichtung so angeordnet ist, dass ein Abstand zwischen der Kühlvorrichtung und dem Herausgabeanschluss kleiner als ein Abstand zwischen der Heizeinheit und dem Herausgabeanschluss ist.

7. Kühlverfahren für einen erhitzten Keramikkörper, bei dem ein Kühlen unter Verwendung einer Kühlvorrichtung durchgeführt wird, die ein Transportelement zum Transportieren einer Heizeinrichtung, in der ein erhitzter Keramikkörper aufgenommen ist, umfasst,
bei dem
die Kühlvorrichtung ferner eine Vielzahl von Gebläsen umfasst, und
der erhitzte Keramikkörper, der in der Heizeinrichtung aufgenommen ist, die auf dem Transportelement angeordnet ist, mittels der Gebläse gekühlt wird.

8. Kühlverfahren eines erhitzten Keramikkörpers nach Anspruch 7, bei dem
der erhitzte Keramikkörper auf 20 bis 80°C in 30 bis 120 Minuten gekühlt wird.

9. Kühlverfahren eines erhitzten Keramikkörpers nach Anspruch 7 oder 8, bei dem
die Kühlvorrichtung einen Saugmechanismus zum Absaugen des Innenbereichs der Kühlvorrichtung umfasst.

10. Kühlverfahren eines erhitzten Keramikkörpers nach einem der Ansprüche 7 bis 9, bei dem
die Vielzahl der Gebläse an beiden Seiten bezüglich des Transportelements angeordnet sind.

11. Kühlverfahren eines erhitzten Keramikkörpers nach Anspruch 9 oder 10, bei dem
der Saugmechanismus an der oberen Seite bezüglich des Transportelements angeordnet ist.

12. Kühlverfahren eines erhitzten Keramikkörpers nach einem der Ansprüche 9 bis 11, bei dem
die Kühlvorrichtung ferner ein Entfernungselement zum Entfernen von Ablagerungen umfasst, die an der Heizeinrichtung anhaften.

13. Verfahren zur Herstellung eines Wabenstrukturkörpers, das umfasst:
Herstellen eines säulenförmigen geformten Wabenkörpers, der eine große Anzahl von Zellen aufweist, die longitudinal parallel zueinander mit einer Zellwand dazwischen angeordnet sind, durch Ausformen eines Keramikrohmaterials;
Erhitzen des geformten Wabenkörpers in einer Heizeinrichtung, um einen Wabenstrukturkörper, der einen erhitzten Wabenkörper umfasst, herzustellen und
ferner umfassend:
Vorbereiten einer Kühlvorrichtung, die ein
Transportelement zum Transportieren der Heizeinrichtung; und
eine Vielzahl von Gebläsen umfasst; und
Kühlen des erhitzten Wabenkörpers unter Verwendung der Kühlvorrichtung nach dem Erhitzen des geformten Wabenkörpers in der Heizeinrichtung.

14. Verfahren zur Herstellung eines strukturierten Wabenkörpers nach Anspruch 13,
bei dem der geformte Wabenkörper in einer Heizeinrichtung unter Verwendung eines Heizofens, der die Kühlvorrichtung umfasst, erhitzt und gekühlt wird.

15. Verfahren zur Herstellung eines strukturierten Wabenkörpers nach Anspruch 13 oder 14,
bei dem das Kühlen den erhitzten Keramikkörper auf 20 bis 80°C in 30 bis 120 Minuten kühlt.

16. Verfahren zur Herstellung eines strukturierten Wabenkörpers nach einem der Ansprüche 13 bis 15, bei dem
die Kühlvorrichtung einen Saugmechanismus zum Absaugen des Innenbereichs der Kühlvorrichtung umfasst.

17. Verfahren zur Herstellung eines strukturierten Wabenkörpers nach einem der Ansprüche 13 bis 16, bei dem
die Vielzahl von Gebläsen an beiden Seiten bezüglich des Transportelements angeordnet sind.

18. Verfahren zur Herstellung eines strukturierten Wabenkörpers nach einem der Ansprüche 13 bis 17, bei dem
der Saugmechanismus an der oberen Seite bezüglich des Transportelements angeordnet ist.

19. Herstellungsverfahren für einen strukturierten Wabenkörper nach einem der Ansprüche 13 bis 18, bei dem
die Kühlvorrichtung ferner ein Entfernungselement zum Entfernen von Ablagerungen umfasst, die an der Heizeinrichtung anhaften.

## Revendications

1. Appareil de refroidissement pour un corps cuit, comprenant:
un organe de transport pour transporter un gabarit de cuisson dans lequel un corps cuit en céramique est reçu;
une pluralité de soufflantes pour refroidir ledit corps cuit en céramique; et
un mécanisme d'aspiration pour changer l'atmosphère à l'intérieur dudit gabarit de cuisson d'une atmosphère à gaz inerte en une atmosphère à air.

2. Appareil de refroidissement pour un corps cuit selon la revendication 1,
dans lequel
ladite pluralité de soufflantes sont placées des deux côtés par rapport audit organe de transport.

3. Appareil de refroidissement pour un corps cuit selon la revendication 1 ou 2,
dans lequel
ledit mécanisme d'aspiration est placé sur le côté supérieur par rapport audit organe de transport.

4. Appareil de refroidissement pour un corps cuit selon l'une quelconque des revendications 1 à 3,
comprenant en plus:
un organe d'élimination permettant d'éliminer des dépôts adhérant audit gabarit de cuisson.

5. Appareil de refroidissement pour un corps cuit selon l'une quelconque des revendications 1 à 4,
qui est installé dans un four de cuisson ou à côté d'un orifice de sortie du four de cuisson.

6. Four de cuisson comprenant:
un organe transport pour transporter un gabarit de cuisson dans lequel un corps moulé en céramique est reçu d'un orifice d'entrée vers un orifice de sortie;
une unité de chauffage pour chauffer ledit corps moulé en céramique; et
l'appareil de refroidissement pour un corps cuit divulgué dans l'une quelconque des revendications 1 à 4,
ledit appareil de refroidissement disposé de telle sorte qu'une distance entre ledit appareil de refroidissement et ledit orifice de sortie est inférieure à une distance entre ladite unité de chauffage et ledit orifice de sortie.

7. Procédé de refroidissement d'un corps cuit en céramique dans lequel le refroidissement est exécuté en utilisant un appareil de refroidissement comprenant un organe de transport pour transporter un gabarit de cuisson dans lequel un corps cuit en céramique est reçu,
dans lequel
ledit appareil de refroidissement comprend en plus une pluralité de soufflantes, et
un corps cuit en céramique qui est reçu à l'intérieur du gabarit de cuisson placé sur ledit organe de transport est refroidi par lesdites soufflantes.

8. Procédé de refroidissement d'un corps cuit en céramique selon la revendication 7,
dans lequel
ledit corps cuit en céramique est refroidi dans la plage de 20 à 80°C en 30 à 120 minutes.

9. Procédé de refroidissement d'un corps cuit en céramique selon la revendication 7 ou 8,
dans lequel
ledit appareil de refroidissement comprend un mécanisme d'aspiration pour aspirer la zone intérieure de l'appareil de refroidissement.

10. Procédé de refroidissement d'un corps cuit en céramique selon l'une quelconque des revendications 7 à 9,
dans lequel
ladite pluralité de soufflantes sont placées des deux côtés par rapport audit organe de transport.

11. Procédé dé refroidissement d'un corps cuit en céramique selon la revendication 9 ou 10,
dans lequel
ledit mécanisme d'aspiration est placé sur le côté supérieur par rapport audit organe de transport.

12. Procédé de refroidissement d'un corps cuit en céramique selon l'une quelconque des revendications 9 à 11,
dans lequel
ledit appareil de refroidissement comprend en plus un organe d'élimination permettant d'éliminer des dépôts adhérant audit gabarit de cuisson.

13. Procédé pour fabriquer un corps à structure en nid d'abeille, comprenant:
la fabrication d'un corps moulé en nid d'abeille en forme de colonne ayant un grand nombre de cellules placées longitudinalement en parallèle les unes aux autres avec une paroi cellulaire entre elles, en moulant une matière première en céramique;
la cuisson dudit corps moulé en nid d'abeille dans un gabarit de cuisson pour fabriquer un corps à structure en nid d'abeille comprenant un corps cuit en nid d'abeille, et
comprenant en plus:
la préparation d'un appareil de refroidissement comprenant
un organe de transport pour transporter ledit gabarit de cuisson; et
une pluralité de soufflantes; et
le refroidissement du corps cuit en nid d'abeille en utilisant ledit appareil de refroidissement après ladite cuisson dudit corps moulé en nid d'abeille à l'intérieur du gabarit de cuisson.

14. Procédé pour fabriquer un corps à structure en nid d'abeille selon la revendication 13,
dans lequel
ledit corps moulé en nid d'abeille est cuit et refroidit dans un gabarit de cuisson en utilisant un four de cuisson comprenant l'appareil de refroidissement.

15. Procédé pour fabriquer un corps à structure en nid d'abeille selon la revendication 13 ou 14,
dans lequel
ledit refroidissement refroidit le corps cuit en céramique de 20 à 80°C pendant 30 à 120 minutes.

16. Procédé pour fabriquer un corps à structure en nid d'abeille selon l'une quelconque des revendications 13 à 15,
dans lequel
ledit appareil de refroidissement comprend un mécanisme d'aspiration pour aspirer la zone intérieure de l'appareil de refroidissement.

17. Procédé de fabriquer un corps à structure en nid d'abeille selon l'une quelconque des revendications 13 à 16,
dans lequel
ladite pluralité de soufflantes sont placées aux deux côtés par rapport audit organe de transport.

18. Procédé pour fabriquer un corps à structure en nid d'abeille selon l'une quelconque des revendications 13 à 17,
dans lequel
ledit mécanisme d'aspiration est placé au côté supérieur par rapport audit organe de transport.

19. Procédé pour fabriquer un corps à structure en nid d'abeille selon l'une quelconque des revendications 13 à 18,
dans lequel
ledit appareil de refroidissement comprend en plus un organe d'élimination permettant d'éliminer des dépôts adhérant audit gabarit de cuisson.
